

## UNITED STATES PATENT OFFICE

2,166,103

## ART OF TREATING FATTY OILS

Otho M. Behr, Redondo Beach, Calif., assignor  
to Vegetable Oil Products Company, Inc., Los  
Angeles, Calif., a corporation of Delaware

No Drawing. Application May 10, 1937,  
Serial No. 141,881

8 Claims. (Cl. 260—428)

This invention relates to the treatment of fatty oils such as vegetable, marine and animal oils and is particularly directed to a process of treating oils containing mixtures of unsaturated and saturated fatty acids or glycerides to the end that distinct liquid products be produced therefrom, these products being particularly adapted for use in the paint, lacquer, varnish and linoleum industries or for use as edible oils 10 or wherever a non-drying oil is required.

The invention also relates to drying oils characterized by their ability to polymerize and/or condense very readily, these oils being further characterized by their ability to form, upon being heated, a true irreversible gel without exhibiting syneresis, and by their ability to form extremely hard, quick-drying films which are extremely stable to weather, alkalies, or the like.

Vegetable, marine and other similar oils are generally classified as drying or non-drying, these being relative terms which to a certain extent indicate the proportionate amount of unsaturated constituents in the oil. For example, the iodine value normally assigned to such oils is a measure of unsaturation and is closely associated with the ability of the oil to absorb oxygen and this in turn is indicative of the drying power of the oil. As a result, it may be generally stated that the more unsaturated oils are drying oils whereas those which contain saturated compounds are non-drying. Linseed oil is an example of what is known as a drying oil whereas cottonseed oil is a substantially non-drying oil. Saturated and partly saturated oils 35 are usually employed and referred to as edible oils, the more unsaturated being generally considered as drying or non-edible.

In addition to the oils which fall into the above general classification, there are oils which contain both saturated and unsaturated compounds and thereby partake of the characteristics of both of the groups. Fish oil, such as sardine oil, for example, contains triglycerides of some very unsaturated acids such as clupanodonic, 45 but the oil also contains relatively high proportions of saturated compounds. Sardine oil per se is not a drying oil because of the presence of the saturated and partly saturated compounds and films of this oil will not dry to a hard, dense 50 film but instead remain tacky. The oil is therefore not suited for use in good paints nor is it entirely edible.

The present invention is primarily directed toward a process whereby a semi-drying oil (or any oil containing saturated, partially saturated and

unsaturated compounds) may be treated to produce two separate and distinct liquid products, each of these products having properties which render it eminently suited for use in a separate and distinct field. A fish oil such as sardine oil, 5 for example, may be converted in accordance with the process of this invention into two fractions, one of which is eminently suited for use in paints, varnishes and the like and has all of the valuable properties of a splendid drying oil such 10 as China-wood oil, for example, whereas the other fractions or product is eminently suited for use either as an edible oil or for hydrogenation, saponification, or the like.

It has been discovered that certain organic 15 solvents, although soluble in vegetable or marine oils, when not added thereto in excess (as for example in less than equal volume), have the property of producing remarkable and unexpected results when added to such oils in ex- 20 cess, i. e., in amounts of more than one volume to one volume of oil. When used in such amounts (preferably more than four volumes to one of oil), these solvents cause a selective precipitation or stratification of certain constituents of the 25 oil, thereby permitting these constituents to be readily withdrawn. In practice, the constituents contained in the settled or precipitated oily layer by action of the solvents are the polymerization and/or condensation products of the 30 unsaturated triglycerides. These polymers and condensation products which are contained in the oily liquid separated from the oils in the manner described, have the property of gelling completely upon being heated so as to form a 35 flexible, resinous gel, whereas most oils which are ordinarily termed good drying oils will not gel completely upon prolonged heating but instead will still exhibit the characteristics of a thick fluid. The two liquid layers obtained by 40 stratification will contain the solvent and portions of liquid oil.

The mixture of oily constituents and solvent which remains after the settled or precipitated liquid portion has been withdrawn may then be 45 separated by distillation into a portion of oil which consists almost essentially of non-drying and saturated components and the original solvent which can then be reused in cyclic operation of the process.

An object of the present invention, therefore, is to disclose and provide a method of treating vegetable, marine and animal oils for the production of separate and distinct liquid products or oils differing greatly in physical and chemical 50 55

properties and adapted for entirely different fields of use.

Another object of this invention is to disclose and provide certain new and useful improved drying oils and methods of producing the same.

A further object of the invention is to disclose and provide a method of manufacturing drying oils which are more waterproof, much harder drying and faster drying, and much more readily 10 and completely polymerized upon further treatment than normal drying oils.

An object of the invention is to disclose and provide a method of producing improved drying oils and improved saturated oils from mixtures 15 thereof.

A still further object of the invention is to disclose and provide a method of precipitating polymerized unsaturated constituents from oils containing the same by means of solvents.

20 These and other objects, uses, advantages and adaptations of the invention will become apparent to those skilled in the art from the following detailed description of the process, ingredients to be used therein, and products produced thereby. It is to be understood that the invention is not limited to the specific examples hereinabove referred to, specific materials and products being mentioned for purposes of illustration only.

In order to facilitate understanding of the invention, the process of this invention will be described as it may be used in the treatment 30 of sardine oil, which is a semi-drying oil incapable of being used in quality paints and varnishes because it does not dry to a hard film but instead 35 remains tacky and contains both saturated and unsaturated triglycerides. Although this and other oils may be subjected to the process of this invention in their normal condition or form, it is preferable in most instances to first subject 40 the oil to a preliminary heating operation for the purpose of polymerizing or heat-bodying the oil. Sardine oil, for example, may be polymerized at temperatures of 525° F.-565° F. Temperatures of from about 480° F. to about 600° F.-45 610° F. may be used, however. By heating this oil under vacuum, a lighter color is maintained. The heat-bodying is carried out to cause simple 50 polymerization with no, or only a minimum, of gel formation and this control is attained by observing the drop in iodine value. The iodine value should not be reduced to a minimum but instead the heat-bodying treatment stopped at

a suitable solvent such as acetone, the solvent being preferably added to the oil during agitation. It will be noted that up to about one volume of acetone may be added to and dissolved in the oil. The addition of acetone is continued, however, (with continuing agitation) until two or more volumes of acetone have been added. In practice, nine to twelve volumes of acetone have been used but four to seven volumes are generally sufficient, particularly when the oil and solvent are heated to temperatures approaching the boiling point of the solvent. After such addition, agitation is discontinued and the resulting mixture permitted to stratify. It will be found that a certain quantity of oil will settle to the bottom of the container. After two to eight hours the settled or precipitated liquid oil is drained off in any suitable manner and it will be found that this precipitated oil is composed essentially of unsaturated polymers but contains 20 from about 20% to 25% of acetone in solution therein. This withdrawn settled oil is then heated to drive off the acetone dissolved therein or again treated with nine or more volumes of acetone. In the event retreatment is not desired, the small amount of acetone remaining in solution in the settled or precipitated oil is removed by distillation or heating and the residual liquid polymerized oil is now ready for use in 25 paints, varnishes, linoleum or wherever a high 30 quality drying oil is desired.

The mixture or upper layer, composed largely of acetone, remaining in the mixer is now distilled for the purpose of recovering the acetone 35 and it will be found that the residual oil obtained from this distillation is composed essentially of partially saturated compounds and is eminently suited for use either as an edible oil, in shortening, or in the manufacture of soaps 40 and other products in which the non-drying oils are ordinarily used. As a specific example, an alkali refined bleached winterized sardine oil was heat-polymerized to Gardner Holdt X viscosity 45 (12.9 poises at 25° C.) and then treated with two 10% extractions with acetone, i. e., nine volumes of acetone to one volume of oil in each extraction. The characteristics of the original 50 sardine oil, after being heat-bodied, and the characteristics and properties of the settled, liquid unsaturated polymer and of the non-drying saturated oil obtained in accordance with this invention are given in the following table:

|    |                                  | Original oil    | Heat bodied oil | Settled polymerized oil | Non-drying oil |    |
|----|----------------------------------|-----------------|-----------------|-------------------------|----------------|----|
| 55 |                                  |                 |                 |                         |                | 55 |
|    | Iodine value Wijs                | 201             | 112             | 118.3                   | 100.9          |    |
|    | Refractive index at 25° C.       | 1.4795          | 1.4933          | 1.4926                  | 1.4872         |    |
| 60 | Saponification value             | 180             | 190             | 185                     | 197            |    |
|    | Free fatty acid as oleic percent | 0.2             | 1.66            | 0.28                    | 3.8            |    |
|    | Color (Lovibond)                 | 35Y/2.5R        | 35Y/4.0R        | 35Y/4.0R                | Greenish       | 60 |
|    | Unsaponifiable percent           | 1               | 1               | 1                       | 0.92           |    |
|    | Viscosity                        | A               | X               | Z5 plus                 | G              |    |
|    | Appearance                       | Cloudy          | Cloudy          | Cloudy                  | Cloudy         |    |
|    | Ability to gel on heating        | No              | No              | Yes                     | No             |    |
|    | Drying                           | Fast, but tacky | Slow, and tacky | Fast                    | Non-drying     |    |
|    | Surface                          |                 |                 | Hard                    | Do             |    |
| 65 | Water resistance                 | Poor            | Poor            | Excellent               | Poor           |    |
|    | Taste                            | Fishy           | Burnt           | Cooked                  | Tasteless      | 65 |
|    | Odor                             | do              | Cooked          | Odorless                | Odorless       |    |

such a point that the oil, at some subsequent time, is capable of exhibiting a further and appreciable drop in iodine value upon further heating. The resulting heat-bodied oil contains a mixture of polymerized unsaturated compounds and unpolymerized saturated constituents.

This heat-bodied sardine oil at atmospheric or superatmospheric temperatures is mixed with

70 The oil obtained by this process and containing the polymerization or condensation products, is distinguishable by its markedly improved drying and film characteristics, such as increased waterproofness and weather resistance, hardness and tenacity of film, speed of drying, and by the fact that it polymerized more readily and to a further extent under the influence of heat. 75

This last property is of great value and permits the use of the product in varnishes as well as in other products requiring the presence of a desirable drying oil that will form an irreversible 5 gel on further heating. The condensation products of this invention will gel completely and can be used as substitutes for China-wood oil, with improved results in many cases.

The partially saturated edible oil (recovered 10 from the solvent) can be neutralized, deodorized, and rendered tasteless by any normal treatment, such as agitation with steam under vacuum, and at temperatures as high as 450° F., without becoming heavy in body. This oil can be used in 15 edible products, while ordinary sardine oils can not unless hydrogenated.

The original oil subjected to the treatment may or may not be heat-bodied prior to treatment, although best results are obtained when the 20 original oil is heat-bodied to a point wherein maximum polymerization has occurred with a minimum of gel formation. This optimum point can be determined by plotting the curve of the 25 viscosity, specific gravity, refractive index or iodine value against time, temperature or both. This curve will be found to change rapidly when the proper polymerization temperature is reached and will then flatten out. I have found the optimum point is where the curve changes from 30 the steep slope to the flatter portion.

Various solvents or liquid precipitants can be used. In general, it appears desirable that the solvent be capable of dissolving, to some extent, in the mixed oil. The solvent should not exert 35 a solvent action upon triglycerides of high molecular weight, such as 900 or more. Ketones and the higher alcohols appear to be usable, and dimethyl ketone, methyl ethyl ketone, diethyl ketone, and higher ketones, such as diacetone, 40 butyl and amylic alcohol, primary hexyl, secondary amyl, hexyl, tetrahydrofurfuryl alcohol and other higher alcohols in primary, secondary and tertiary forms are examples. Alcohols of higher molecular weight (from those mentioned) give 45 better results than those of lower molecular weight. Most of the aliphatic hydrocarbons, chlorinated aliphatics and aromatics are not effective.

The volume of solvent used should be at least 50 three or four times, and preferably seven to twelve times, the volume of the oil. The mixing and precipitation can be carried out at atmospheric or superatmospheric temperatures. By using heat during mixing and stratification or 55 precipitation, a more effective precipitation is attained. The precipitated oils can be caused to separate by gravity or by the aid of centrifugal separators. The entire process may be batch or of the continuous counterflow type. By varying 60 the ratio of solvent to oil, degree of initial polymerization, temperature of extraction and/or the number of extractions carried out on the heavier oil, great latitude in the character of the precipitated and residual oils may be obtained. In this 65 manner, the products made may be controlled to meet market demands.

Those skilled in chemical engineering and oil processing will readily appreciate the variety of devices which can be used in carrying out the 70 process of this invention, and for this reason a specific exemplary form is not described in detail.

I claim:

1. A method of treating partially polymerized 75 vegetable and marine oils containing polymers of unsaturated constituents in liquid phase and not

as solid gels, the oils being capable of exhibiting a drop in iodine value upon heat-bodying, to produce an oil fraction having enhanced drying properties, comprising: mixing a given volume of such partially polymerized oil with not less than three volumes of an organic solvent from the group consisting of ketones and higher alcohols, permitting the mixture to settle and stratify into two layers, each containing a solution of oily constituents and solvent, separating the bottom layer containing polymerized constituents having enhanced drying properties from the upper layer, and separating solvent from the upper layer to obtain a substantially non-drying oil.

2. A method of treating partially polymerized 15 vegetable and marine oils containing polymers of unsaturated constituents in liquid phase and not as solid gels, the oils being capable of exhibiting a drop in iodine value upon heat-bodying, to produce an oil fraction having enhanced dry- 20 properties, comprising: mixing a given volume of such partially polymerized oil with not less than three volumes of an organic solvent from the group consisting of ketones and higher alcohols, permitting the mixture to settle and 25 stratify into two layers, each containing a solution of oil and solvent, separating the settled bottom layer of solution containing polymerized constituents from the supernatant liquid, said bottom layer containing oil having enhanced dry- 30 properties, separating the solvent from the supernatant liquid to obtain an oil fraction having substantially non-drying properties, and removing solvent from the bottom layer.

3. A method of treating vegetable and marine 35 oils to recover therefrom oil fractions having enhanced drying properties, comprising: subjecting the oil to an incomplete polymerizing treatment virtually insufficient to form solid gels, the partially polymerized oil being capable of exhibiting a drop in iodine value upon further heat- 40 bodying; mixing said partially polymerized oil with not less than three volumes of an organic solvent from the group of ketones and higher alcohols; separating the mixture gravimetrically 45 into two layers of solution of oil and solvent, recovering a liquid oil fraction having enhanced drying properties from one layer and recovering an oil fraction having non-drying characteristics from the other layer.

4. A method of treating vegetable and marine 50 oils to recover therefrom oil fractions having enhanced drying properties, comprising: subjecting the oil to an incomplete polymerizing treatment virtually insufficient to form solid gels, the partially polymerized oil being capable of exhibiting a drop in iodine value upon further heat- 55 bodying; mixing said partially polymerized oil with not less than three volumes of an organic solvent from the group of ketones and higher alcohols; separating the mixture gravimetrically 60 into two layers of solution of oil and solvent, separating organic solvents from each of said layers separately, recovering an oil fraction having enhanced drying properties from one layer, and 65 recovering a liquid oil fraction having non-drying characteristics from the other layer.

5. A method of treating vegetable and marine 70 oils to recover therefrom oil fractions having enhanced drying properties, comprising: subjecting the oil to a partial polymerizing treatment virtually insufficient to form solid gels, the partially polymerized oil being capable of exhibiting a drop in iodine value upon further heat-bodying; mix- 75 ing said partially polymerized oil with not less

- than three volumes of acetone; separating the mixture gravimetrically into two layers, each comprising a solution of oil and solvent; recovering an oil fraction having enhanced drying properties from one layer, and recovering a liquid oil fraction having non-drying characteristics from the other layer.
6. A method of treating partially polymerized vegetable and marine oils to recover therefrom oil fractions having enhanced drying properties, comprising: mixing a partially polymerized oil with not less than three volumes of acetone; separating the mixture gravimetrically into two layers of solution of oil and acetone; separating acetone from each of said solutions separately, recovering an oil fraction having enhanced drying properties from one layer and recovering a liquid oil fraction having non-drying characteristics from the other layer.
- 10 7. In a method of treating partially polymerized vegetable and marine oils containing polymers of unsaturated constituents, the steps of: mixing a given volume of such partially polymerized oil with more than four volumes of an organic solvent from the group consisting of ketones and higher
- 15 alcohols, permitting the mixture to stratify into two layers, each comprising a solution of oily constituents and solvent, separating solvent from each of said layers, recovering a liquid oil containing polymerized constituents and having enhanced drying properties from one layer, and recovering a liquid oil having non-drying characteristics from the other layer.
- 19 8. A method of treating fish oils comprising: subjecting fish oil to a partial polymerizing treatment virtually insufficient to form solid gels, the partially polymerized oil being capable of exhibiting a drop in iodine value upon further heat-bodying; mixing said partially polymerized fish oil with not less than three volumes of an organic solvent from the group of ketones and higher alcohols; separating the mixture gravimetrically into two layers of solution of oil and solvent, separating organic solvents from each of said layers separately, recovering a liquid oil having enhanced drying properties from one layer, and recovering a liquid oil having non-drying characteristics from the other layer.

OTHO M. BEHR. 25